



US006287400B1

(12) **United States Patent**  
Burns et al.

(10) **Patent No.:** US 6,287,400 B1  
(45) **Date of Patent:** Sep. 11, 2001

(54) **GAS GENERANT COMPOSITION**(75) Inventors: **Sean P. Burns**, Almont; **Pares S. Khandhadia**, Troy, both of MI (US)(73) Assignee: **Automotive Systems Laboratory, Inc.**, Farmington Hills, MI (US)

(\*) Notice: Subject to any disclaimer, the term of this patent is extended or adjusted under 35 U.S.C. 154(b) by 0 days.

(21) Appl. No.: **09/516,067**(22) Filed: **Mar. 1, 2000****Related U.S. Application Data**

(60) Provisional application No. 60/122,234, filed on Mar. 1, 1999, and provisional application No. 60/128,101, filed on Apr. 7, 1999.

(51) **Int. Cl.** <sup>7</sup> ..... **C06B 47/08**(52) **U.S. Cl.** ..... **149/36**(58) **Field of Search** ..... 149/36, 46, 47(56) **References Cited**

## U.S. PATENT DOCUMENTS

|           |           |                  |            |
|-----------|-----------|------------------|------------|
| 3,734,789 | 5/1973    | Moy et al.       | 149/19     |
| 3,779,822 | 12/1973   | Stammler et al.  | 149/19.4   |
| 3,845,970 | * 11/1974 | Herrmann         | 280/150 AB |
| 3,898,112 | 8/1975    | Strecker et al.  | 149/19.9   |
| 3,940,298 | * 2/1976  | Beckert et al.   | 149/92     |
| 3,954,528 | 5/1976    | Chang et al.     | 149/19.4   |
| 4,931,112 | 6/1990    | Wardle et al.    | 149/88     |
| 5,386,775 | 2/1995    | Poole et al.     | 102/289    |
| 5,460,668 | 10/1995   | Lyon             | 149/36     |
| 5,514,230 | * 5/1996  | Khandhadia       | 149/36     |
| 5,516,377 | 5/1996    | Highsmith et al. | 149/18     |
| 5,545,272 | 8/1996    | Poole et al.     | 149/48     |

|           |           |                  |         |
|-----------|-----------|------------------|---------|
| 5,684,269 | 11/1997   | Barnes et al.    | 149/45  |
| 5,756,929 | 5/1998    | Lundstrom et al. | 149/22  |
| 5,847,315 | * 12/1998 | Katzakian et al. | 149/36  |
| 5,872,329 | 2/1999    | Burns et al.     | 149/36  |
| 5,924,640 | * 7/1999  | Hickey et al.    | 242/374 |
| 6,024,812 | 2/2000    | Bley et al.      | 149/92  |
| 6,074,502 | 6/2000    | Burns et al.     | 149/36  |
| 6,077,371 | 6/2000    | Lundstrom et al. | 149/37  |
| 6,136,114 | * 10/2000 | Johnson et al.   | 149/22  |

## FOREIGN PATENT DOCUMENTS

Sho  
59-248688 11/1984 (JP).

## OTHER PUBLICATIONS

The Nitration of 5-Aminotetrazole; Journal of Organic Chemistry; R. M. Herbst and J. A. Garrison; 1953.

\* cited by examiner

Primary Examiner—Michael J. Carone

Assistant Examiner—Francis T. Palo

(74) Attorney, Agent, or Firm—Laurence C. Begin; Dinnin &amp; Dunn PC

(57)

## ABSTRACT

Preferred gas generant compositions incorporate a combination of 5-aminotetrazole nitrate and an oxidizer. The oxidizer may be selected from a group including nonmetal and metal nitrates, nitrites, chlorates, chlorites, perchlorates, and oxides. 5-aminotetrazole nitrate is characterized as an oxygen-rich fuel and is therefore considered to be a self-deflagrating fuel. To tailor the oxygen balance in certain applications, however, the use of an oxidizer is preferred. These compositions are especially suitable for inflating air bags and actuating seatbelt pretensioners in passenger-restraint devices.

9 Claims, 4 Drawing Sheets









Fig. 3



**GAS GENERANT COMPOSITION****CROSS REFERENCE TO RELATED APPLICATIONS**

This application claims the benefit of U.S. Provisional Application Numbers 60/122,234 and 60/128,101, filed on Mar. 1, 1999 and Apr. 7, 1999, respectively.

**BACKGROUND OF THE INVENTION****FIELD OF THE INVENTION**

The present invention relates to nontoxic gas generating compositions that when combusted rapidly generate gases that are useful for actuating vehicle occupant restraint systems in motor vehicles and specifically, the invention relates to thermally stable nonazide gas generants having not only acceptable burn rates and sustained combustion, but also a relatively high gas volume to solid particulate ratio at acceptable flame temperatures.

The evolution from azide-based gas generants to nonazide gas generants is well-documented in the prior art. The advantages of nonazide gas generant compositions in comparison with azide gas generants have been extensively described in the patent literature, for example, U.S. Pat. Nos. 4,370,181; 4,909,549; 4,948,439; 5,084,118; 5,139,588, 5,035,757, 5,386,775, and 5,872,329, the discussions of which are hereby incorporated by reference.

In addition to a fuel constituent, pyrotechnic nonazide gas generants contain ingredients such as oxidizers to provide the required oxygen for rapid combustion and reduce the quantity of toxic gases generated, a catalyst to promote the conversion of toxic oxides of carbon and nitrogen to innocuous gases, and a slag forming constituent to cause the solid and liquid products formed during and immediately after combustion to agglomerate into filterable clinker-like particulates. Other optional additives, such as burning rate enhancers or ballistic modifiers and ignition aids, are used to control the ignitability and combustion properties of the gas generant.

One of the disadvantages of known nonazide gas generant compositions is the amount and physical nature of the solid residues formed during combustion. The solids produced as a result of combustion must be filtered and otherwise kept away from contact with the occupants of the vehicle. It is therefore highly desirable to develop compositions that produce a minimum of solid particulates while still providing adequate quantities of a nontoxic gas to inflate the safety device at a high rate.

The use of phase stabilized ammonium nitrate is desirable because it generates abundant nontoxic gases and minimal solids upon combustion. To be useful, however, gas generants for automotive applications must be thermally stable.

Often, gas generant compositions incorporating phase stabilized or pure ammonium nitrate exhibit poor thermal stability, and produce unacceptably high levels of toxic gases, CO and NO<sub>x</sub> for example, depending on the composition of the associated additives such as plasticizers and binders. In addition, ammonium nitrate contributes to poor ignitability, lower burn rates, and performance variability. Several known gas generant compositions incorporating ammonium nitrate utilize well-known ignition aids such as BKNO<sub>3</sub> to solve this problem. However, the addition of an ignition aid such as BKNO<sub>3</sub> is undesirable because it is a highly sensitive and energetic compound, and furthermore, contributes to thermal instability and an increase in the amount of solids produced.

Certain gas generant compositions comprised of ammonium nitrate are thermally stable, but have burn rates less

than desirable for use in gas inflators. To be useful for passenger restraint inflator applications, gas generant compositions generally require a burn rate of at least 0.4 inch/second (ips) or more at 1000 psi. Gas generants with burn rates of less than 0.40 ips at 1000 psi do not ignite reliably and often result in "no-fires" in the inflator.

Yet another problem that must be addressed is that the U.S. Department of Transportation (DOT) regulations require "cap testing" for gas generants. Because of the sensitivity to detonation of fuels often used in conjunction with ammonium nitrate, most propellants incorporating ammonium nitrate do not pass the cap test unless shaped into large disks, which in turn reduces design flexibility of the inflator.

The compositions described in U.S. Pat. No. 5,035,757 to Poole exemplify state of the art gas generant compositions that function well but produce relatively large amounts of solid combustion products. As a result, the gas produced is less than that produced by current state of the art "smokeless" gas generants. Thus, more gas generant and greater filtering requirements are required during operation of an airbag inflator.

On the other hand, compositions described in U.S. Pat. No. 5,872,329 to Burns et al. exemplify current state of the art "smokeless" gas generants. The combustion products are primarily gas with minimal formation of solids. The benefits include a reduction in the amount of gas generant required and reduced filtering requirements. However, these compositions may be disadvantaged by lower burn rates and a failure to sustain gas generant combustion. To overcome these disadvantages, a stronger and more robust inflator is often required to increase the operating pressure of the inflator and thereby improve the burn of the gas generant.

Accordingly, it would be an improvement in the art to provide the gas generant burn characteristics of compounds as described in U.S. Pat. No. 5,035,757 along with the capacity to produce more gas and less solids as exhibited by state of the art "smokeless" gas generants.

**SUMMARY OF THE INVENTION**

The present invention generally relates to gas generant compositions useful in actuating a vehicle occupant restraint system in the event of a motor vehicle accident. Application within a vehicle occupant restraint system includes actuation of a seatbelt pretensioner and/or inflation of an airbag. Other applications requiring gas generation are also contemplated, including fire suppression systems aboard aircraft and inflators for flotation devices, for example.

The above-referenced problems are reconciled by compositions containing 5-aminotetrazole nitrate (5ATN) as a fuel at about 25-100% by weight of the total composition.

An oxidizer is selected from a group of compounds including phase stabilized ammonium nitrate, ammonium nitrate, potassium nitrate, strontium nitrate, copper dioxide, and basic copper nitrate. Other oxidizers well known in the art are also contemplated. These generally include but are not limited to inorganic oxidizers such as alkali and alkaline earth metal nitrates, nitrites, chlorates, chlorites, perchlorates, and oxides.

Standard binders, slag formers, and coolants may also be incorporated if desired.

A composition in accordance with the present invention contains by weight 25-95% 5ATN and 5-75% of an oxidizer. A more preferred composition consists of 55-85% 5ATN and 20-45% PSAN.

**BRIEF DESCRIPTION OF THE FIGURES**

FIG. 1 illustrates the burn rate of state of the art "smokeless" gas generants as compared to a preferred embodiment of the present invention.

FIG. 2 illustrates the 60L tank pressure and chamber pressure resulting from combustion of state of the art "smokeless" gas generants and a preferred embodiment of the present invention.

FIG. 3 illustrates a comparison of pressure vs. time in a 40 cc tank with respect to state of the art compositions, preferred embodiments of the present invention and control compositions.

FIG. 4 illustrates the melting point and decomposition temperatures of a preferred embodiment of the present invention, as well as related data separately comparing the respective constituents of the preferred embodiment.

FIG. 5 illustrates the autoignition temperature of a preferred embodiment of the present invention.

#### DESCRIPTION OF THE PREFERRED EMBODIMENTS

The gas generants of the present invention when compared to other state of the art gas generants ignite easier, produce minimal solids, exhibit improved burn rates, are thermally stable, and sustain a burn at lower pressures.

In accordance with the present invention, 5-aminotetrazole nitrate (5-ATN) is provided at 25–100% by weight of the gas generant, depending on the application. 5-ATN is characterized as an oxygen-rich fuel attributed to the oxygen in the nitrate group. The use of 5-ATN within a gas generant composition therefore requires little or no additional oxidizer, again depending on the application. 5-ATN is more preferably provided at 30–95% by weight and most preferably provided at 55–85% by weight of the gas generant composition.

In certain applications, the oxygen balance must be tailored to accommodate reduced levels of carbon monoxide (CO) and nitrogen oxides (NO<sub>x</sub>) as driven by original equipment manufacturer toxicity requirements. For example, the gas generated upon combustion of a gas generant within a vehicle occupant restraint system must minimize or eliminate production of these toxic gases. Therefore, when adding an oxidizer to 5-ATN, it is generally understood that an oxygen balance of about -4.0 to +4.0 is desirable when the gas generant is used in an airbag inflator. The preferred percentages of 5-ATN reflect this characteristic.

One or more oxidizers may be selected from the group including nonmetal, alkali metal, and alkaline earth metal nitrates, nitrites, perchlorates, chlorates, and chlorites for example. Other oxidizers well known in the art may also be used. These include alkali, alkaline earth, and transitional metal oxides, for example. Preferred oxidizers include phase stabilized ammonium nitrate (PSAN), ammonium nitrate, potassium nitrate, and strontium nitrate. The oxidizer(s) is provided at 5–70% by weight of the gas generant composition and more preferably at 20–45% by weight of the oxidizer.

Standard additives such as binders, slag formers, burn rate modifiers, and coolants may also be incorporated if desired. Inert components may be included and are selected from the group containing clay, silicon, silicates, diatomaceous earth, and oxides such as glass, silica, alumina, and titania. The silicates include but are not limited to silicates having layered structures such as talc and the aluminum silicates of clay and mica; aluminosilicate; borosilicates; and other silicates such as sodium silicate and potassium silicate. The inert component is present at about 0.1–20% by weight, more preferably at about 0.1–8%, and most preferably at 0.1–3%.

A most preferred embodiment contains 73.12% 5-ATN and 26.88% PSAN10 (stabilized with 10% potassium nitrate). The invention is further exemplified by the following examples.

#### EXAMPLE 1

5ATN was prepared according to the following method. In an ice bath, 20 g (0.235 moles) of anhydrous 5-aminotetrazole and 22 ml (0.350 moles) of concentrated nitric acid were stirred for about one hour. About 70 ml of water was added directly to the slurry, and the entire mixture was heated quickly to boiling. The hot solution was vacuum filtered and allowed to cool at ambient conditions while stirring. The white crystals formed during cooling were vacuum filtered and washed with cold water, then forced through a No. 14 mesh screen to form granules. The wet material was dried for one hour at ambient conditions and formed well-flowing granules.

By TGA, the 5ATN dried at ambient conditions contained about 1.0 wt % water. As tested on a BOE impact apparatus, this material showed no positive fires up to 25 inches (equivalent to about 231 kp.cm).

#### EXAMPLE 2

The 5ATN granules prepared in Example 1 were dried at 105 degrees Celsius for 4 hours to remove any remaining moisture. Elemental analysis for C, H, and N showed by weight 8.36% carbon, 2.71% hydrogen, and 56.71% nitrogen. The theoretical values by weight are 8.11% C, 2.72% H, 56.75% N, and 32.41% O.

As tested on a BOE impact apparatus, this material showed positive fires at about 4 inches (equivalent to about 37 kp.cm). This demonstrates how 5ATN experiences an increase in impact sensitivity when completely dry.

The dried 5ATN was tested using a DSC at a heating rate of 10 degrees Celsius per minute. The 5ATN melted at 156.8 degrees Celsius and then decomposed exothermically with an onset of 177.2 degrees Celsius and a peak of 182.5 degrees Celsius. The 5ATN was also tested using a TGA at a heating rate of 10 degrees Celsius per minute and found to have an 89.3 wt % gas conversion up to 450 degrees Celsius, with a 67.5 wt % gas conversion up to about 194 degrees Celsius. The DSC and TGA data show that the 5ATN autoignites at about 180 degrees Celsius with a large release of energy.

#### EXAMPLE 3

The wet 5ATN granules as prepared in Example 1 were compression molded in a 0.5 inch die under a 10-ton force to a height of about 0.1 inches. About half of the pellets were dried for 4 hours at 70 degrees Celsius to remove all the moisture. A weight loss of about 1.0 wt % confirmed that all of the moisture had been removed.

Both the wet and dry 5ATN pellets were tested as a booster material using the following specifications. Each pellet was broken into four pieces and the fragments were loaded into a small aluminum cup. This aluminum cup was then crimped to a standard air bag initiator that contained 110 mg of zinc potassium perchlorate (ZPP). The entire assembly, known as an igniter, was fired inside a closed bomb with a volume of 40 cubic centimeters. The 40 cubic centimeter bomb was equipped with a pressure transducer to measure the pressure rise over time.

FIG. 3 shows the results of the tests. Other control tests were done as a comparison to the igniters containing 5ATN.

Tests **7** and **8** (initiator) are igniters consisting of an empty aluminum cup crimped to an initiator. Tests **9** and **10** are control igniters containing both an autoignition material and 8 pellets of a standard nonazide composition as described in U.S. Pat. No. 5,035,757. Test **11** is another control igniter similar to tests **9** and **10**, except with autoignition material and 14 pellets of the same nonazide composition. Test **12** is an igniter containing about 0.7g of undried 5ATN pellet fragments. Test **13** is an igniter containing about 1.0 g of undried 5ATN pellet fragments. In all cases, the igniters containing 5ATN ignited readily and actually reached peak pressure sooner than the control igniters. In both tests **11** and **13**, the volume of the aluminum cup was completely full. As shown in FIG. 3, for an equivalent volume of material, the output of the 5ATN igniter (**13**) is about twice that of the control igniter containing the state of the art propellant (**11**).

#### EXAMPLE 4

A composition was prepared containing 77.77 wt. % 5ATN and 22.23 wt. % strontium nitrate. The 5ATN as prepared in Example 1 and dried strontium nitrate were combined to form an overall mass of 0.71 g and then mixed and ground with a mortar and pestle. The composition was tested by DSC at a heating rate of 5 degrees Celsius per minute and found to melt at 155.3 degrees Celsius and then decomposed with a large exotherm (175.6 degrees Celsius onset, 179.4 degrees Celsius peak). The composition was tested by TGA at a heating rate of 10 degrees Celsius per minute and found to have a 91.7 wt. % gas conversion up to 950 degrees Celsius, with a 74.1wt. % gas conversion up to about 196 degrees Celsius. As tested on a BOE impact apparatus, this composition showed positive fires at about 3 inches (equivalent to about 28 kp.cm). This composition burned vigorously when ignited with a propane torch.

#### EXAMPLE 5

A composition was prepared containing 65.05wt. % 5ATN and 34.95 wt. % copper (II) oxide. The 5ATN as prepared in Example 1 and the dried copper oxide were combined to form an overall mass of 0.52 g and then mixed and ground with a mortar and pestle. The composition was tested by DSC at a heating rate of 10 degrees Celsius per minute and found to decompose with a large exotherm peaking at about 175 degrees Celsius. The composition was tested by TGA at a heating rate of 10 degrees Celsius per minute and found to have an 83.4 wt. % gas conversion up to 400 degrees Celsius, with an 80.6 wt. % gas conversion up to about 183 degrees Celsius. As tested on a BOE impact apparatus, this composition showed positive fires at about 3 inches (equivalent to about 28 kp.cm). This composition burned vigorously when ignited with a propane torch.

#### EXAMPLE 6

A composition was prepared containing 65.05wt. % 5ATN and 34.95 wt. % copper (II) oxide. The 5ATN as prepared in Example 1 and the dried copper oxide were combined to form an overall mass of 1.00 g. Enough water was added to form a slurry and then the components were mixed and ground with a mortar and pestle. The water was allowed to evaporate by holding the mixture at 70 degrees Celsius. Eventually, a sticky, polymer-like substance formed which became very hard with complete drying. The composition was tested by DSC at a heating rate of 10 degrees Celsius per minute and found to exhibit multiple exotherms beginning at about 137 degrees Celsius. This composition burned vigorously when ignited with a propane torch. This

example demonstrates how 5ATN can be combined with a common oxidizer through either dry or wet mixing.

#### EXAMPLE 7

A composition was prepared containing 67.01 wt. % 5ATN and 32.99 wt. % PSAN10 (AN phase stabilized with 10 wt. % KN). The 5ATN as prepared in Example 1 and the dried PSAN 10 were combined to form an overall mass of 0.24 g and then mixed and ground with a mortar and pestle. FIG. 5 shows a melting point of 132° C. and a decomposition point of 153° C. See curve 17. The various constituents are also analyzed separately. See curves 14–16.

#### EXAMPLE 8

As FIG. 1 illustrates, gas generants of the present invention as exemplified by curve **1**, have acceptable burn rates at ambient pressures and above, and have significantly higher burn rates as compared to state of the art “smokeless” gas generants (curve **2**). Curve **1** indicates a gas generant containing 73.12 5-ATN and 26.88% phase stabilized ammonium nitrate (stabilized with 10% potassium nitrate). Curve **2** is a comparison of a gas generant containing 65.44% phase stabilized ammonium nitrate (stabilized with 10% potassium nitrate or PSAN10), 25.80% of the diammonium salt of 5,5'-Bi- 1H-tetrazole, 7.46% strontium nitrate, and 1.30% clay. The pressure exponent of the present invention, 0.71 is less than the pressure exponent of the state of the art “smokeless” gas generant of curve **2**, 0.81. As shown in FIG. 2, a typical embodiment autoignites at 147° C. See curve **21**. The gas generant constituents when taken alone do not indicate autoignition from 0–400° C.

#### EXAMPLE 9

FIG. 3 illustrates a comparison between a preferred embodiment containing the same, fuel as curve **1** in Example 8. See curves **3** and **4**. Curves **5** and **6** correspond to the same “smokeless” gas generant as indicated in curve **2** of Example 8. As curves **3** and **5** indicate, the chamber pressure resulting from combustion of the preferred embodiment is at 26 Mpa whereas the chamber pressure of the state of the art “smokeless” gas generant is 37 Mpa. On the other hand, as shown in curves **4** and **6**, the 60L tank pressures are approximately equivalent given the same inflator. The data can be interpreted to show that compositions of the present invention require less pressure but maintain superior burn rates (see FIG. 1) and thus are able to provide approximately equivalent inflation pressure for an airbag. As a result, a less robust inflator with a weaker ignition source may be used in compositions of the present invention. Compare the igniters used in FIG. 3 and Example 3.

#### EXAMPLE 10

Two compositions were prepared and tested. The burn rate was measured by igniting a compressed slug in a closed bomb at a constant pressure of 1000 psi. The ignitability of the formulations was determined by attempting to ignite the samples at ambient pressure with a propane torch. The outputs of the subjective analysis are the following: the time it takes for the sample to reach self-sustaining combustion after the torch flame touches the sample, and the ease of which the sample continues combustion when the torch flame is removed.

Formulation 1 was 73.12% 5-ATN and 26.89% PSAN10. The sample ignited instantly when touched with the flame from a propane torch and continued to burn vigorously when

the flame was removed. The burn rate of this formulation at 1000 psi was measured to 0.69 inches per second (ips). To minimize the production of either CO or NO<sub>x</sub>, this composition was formulated to have an oxygen balance of -2.0 wt. % oxygen.

Formulation 2 was 62.21 % azobisformamidine dinitrate and 37.79% PSAN10. When contacted with the flame from a propane torch, the sample did not ignite for a few seconds. After it appeared that self-sustaining combustion had begun, the torch was removed and the sample extinguished. After igniting the sample a second time, it burned slowly to completion. The burn rate of this formulation at 1000 psi was measured at 0.47 ips. To minimize the production of either CO or NO<sub>x</sub>, this composition was formulated to have an oxygen balance of 0.0 wt. % oxygen.

It is suspected that the nitrated 5-AT fuel ignites more easily and burns faster for the following reasons:

- 1) The base 5-AT fuel has more energy (positive heat of formation) than the base azobisformamidine fuel (negative heat of formation).
- 2) The nitrated 5-AT has a higher oxygen content and therefore allows for the use of a lesser amount of the PSAN oxidizer. It is well known that the higher levels of PSAN will negatively affect the ignitability and burn rate of many propellant compositions.

#### EXAMPLE 11

Table 1 illustrates the problem of thermal instability when typical nonazide fuels are combined with PSAN:

TABLE 1

| Thermal Stability of PSAN - Non-Azide Fuel Mixtures                                                                                          |                                                                                                                                                                                                                                                                                                                                                                                                                             |
|----------------------------------------------------------------------------------------------------------------------------------------------|-----------------------------------------------------------------------------------------------------------------------------------------------------------------------------------------------------------------------------------------------------------------------------------------------------------------------------------------------------------------------------------------------------------------------------|
| Non-Azide Fuel(s) Combined With PSAN                                                                                                         | Thermal Stability                                                                                                                                                                                                                                                                                                                                                                                                           |
| 5-aminotetrazole (5AT)                                                                                                                       | Melts with 108° C. onset and 116° C. peak. Decomposed with 6.74% weight loss when aged at 107° C. for 336 hours. Poole '272 shows melting with loss of NH <sub>3</sub> when aged at 107° C.                                                                                                                                                                                                                                 |
| Ethylene diamine dinitrate, nitroguanidine (NQ)<br>5AT, NQ<br>5AT, NQ quanidine nitrate (GN)<br>GN, NQ                                       | Melts with 103° C. onset and 110° C. peak. Melts with 93° C. onset on 99° C. peak.                                                                                                                                                                                                                                                                                                                                          |
| GN, 3-nitro-1,2,4-triazole (NTA)<br>NQ, NTA<br>Aminoguanidine nitrate<br>1H-tetrazole (1 HT)<br>Dicyandiamide (DCDA)<br>GN, DCDA<br>NQ, DCDA | Melts with 100° C. onset and 112° C. Decomposed with 6.49% weight loss when aged at 107° C. for 336 hours. Melts with 108° C. onset and 110° C. peak.                                                                                                                                                                                                                                                                       |
| 5AT, GN<br>Magnesium salt of 5AT (M5AT)                                                                                                      | Melts with 111° C. onset and 113° C. peak. Melts with 109° C. onset and 110° C. peak. Melts with 109° C. onset and 110° C. peak. Melts with 114° C. onset and 114° C. peak. Melts with 104° C. onset and 105° C. peak. Melts with 107° C. onset and 115° C. peak. Decomposed with 5.66% weight loss when aged at 107° C. for 336 hours. Melts with 70° C. onset and 99° C. peak. Melts with 100° C. onset and 111° C. peak. |

In this example, "decomposed" indicates that pellets of the given formulation were discolored, expanded, fractured, and/or stuck together (indicating melting), making them unsuitable for use in an air bag inflator. In general, any PSAN-nonazide fuel mixture with a melting point of less than 115 C., will decompose when aged at 107 C. As shown, many compositions that comprise well-known nonazide

fuels and PSAN are not fit for use within an inflator due to poor thermal stability. As shown in FIG. 4 curve 17, the melting point of a preferred embodiment is greater than 115 C. (132 C.), thereby indicating that combining 5-ATN with PSAN does not significantly affect the stability of the fuel.

#### EXAMPLE 12

A composition containing 73.12% 5-ATN and 26.88% PSAN10 has been tested for sensitivity with the following results:

|    |                          |          |
|----|--------------------------|----------|
| 15 | Impact (BOE Apparatus)   | 48 kp.cm |
|    | Friction (BAM Apparatus) | 120 N    |
|    | Electrostatic Discharge  | >900 mJ  |

The preferred composition was compared to nitrocellulose, a standard gas generant for seat belt pretensioners. Gas yield, gas conversion, autoignition temperature, solids production, combustion temperatures, and density were roughly equivalent. Seat belt retractor tests also revealed fairly equivalent performance results. The following data was developed relative to nitrocellulose:

|    |                          |          |
|----|--------------------------|----------|
| 30 | Impact (BOE Apparatus)   | 29 kp.cm |
|    | Friction (BAM Apparatus) | >360 N   |
|    | Electrostatic Discharge  | NA       |

The preferred embodiment resulted in combustion gases containing 0.0% CO and 2.4% hydrogen, and 96.7% preferred gases containing nitrogen, carbon dioxide, and water. On the other hand, nitrocellulose resulted in combustion gases containing 29.2% CO and 19.7% hydrogen, and 51.1% preferred gases containing nitrogen, carbon dioxide, and water.

It can therefore be concluded that compositions of the present invention provide similar performance to nitrocellulose but with improved thermal stability, impact sensitivity, and content of effluent gases when used as a pretensioner gas generant.

#### EXAMPLE 13

Compositions containing 100% 5-ATN were used as pretensioner gas generators despite exhibiting an oxygen balance of -10.80 wt. % oxygen. The amount of gas generant used in a pretensioner is small enough (roughly one gram) to permit an excessive negative oxygen balance without prohibitive levels of CO.

#### EXAMPLE 14

As shown in Table 2, other compositions of the present invention include gas generators exhibiting oxygen balances in the range of -11.0 to +11.0. The oxygen balance may be readily determined by well known theoretical calculations. An oxygen balance of about +4.0 to -4.0% is preferred for compositions used in vehicle occupant restraint systems as main gas generators. Compositions exhibiting an oxygen balance outside of this range are useful as autoignition compounds or igniter compounds in an inflator; as a pretensioner gas generant; in a fire suppression mechanism; as a gas generant for an inflatable vessel or airplane ramp, or where levels of toxic gases such as CO and NO<sub>x</sub> are not critical for the desired use.

TABLE 2

| Composition                       | Gas Yield<br>(moles/<br>100 g) | Gas<br>Conversion<br>(wt % to gas) | Gas<br>Products<br>(vol. %)                                                                    | Oxygen<br>Balance<br>(wt % O <sub>2</sub> ) |
|-----------------------------------|--------------------------------|------------------------------------|------------------------------------------------------------------------------------------------|---------------------------------------------|
| Example 5                         | 3.26                           | 89.1                               | 51.6% N <sub>2</sub><br>32.3% H <sub>2</sub> O<br>16.1% CO <sub>2</sub>                        | 0.0                                         |
| Example 6                         | 2.64                           | 72.1                               | 50.0% N <sub>2</sub><br>33.3% H <sub>2</sub> O<br>16.7% CO <sub>2</sub>                        | 0.0                                         |
| 35% 5-ATN<br>41% PSAN10<br>24% NQ | 3.91                           | 98.1                               | 42.3% N <sub>2</sub><br>47.5% H <sub>2</sub> O<br>10.0% CO <sub>2</sub>                        | -2.16                                       |
| 39.4% 5-ATN<br>60.6% PSAN10       | 3.95                           | 97.2                               | 38.2% N <sub>2</sub><br>47.9% H <sub>2</sub> O<br>6.7% CO <sub>2</sub><br>7.2% O <sub>2</sub>  | +9.06                                       |
| 73.1% 5-ATN<br>26.9% PSAN10       | 3.82                           | 98.8                               | 46.4% N <sub>2</sub><br>38.4% H <sub>2</sub> O<br>11.9% CO <sub>2</sub><br>2.4% H <sub>2</sub> | -2.0                                        |
| 60.0% 5-ATN<br>40.0% PSAN10       | 3.87                           | 98.1                               | 43.5% N <sub>2</sub><br>44.2% H <sub>2</sub> O<br>10.5% CO <sub>2</sub><br>1.8% O <sub>2</sub> | +2.3                                        |
| 79.2% 5-ATN<br>20.8% PSAN10       | 3.80                           | 99.0                               | 48.7% N <sub>2</sub><br>37.2% H <sub>2</sub> O<br>14.1% CO <sub>2</sub>                        | -4.0                                        |

The oxygen balance is the weight percent oxygen necessary to result in stoichiometric combustion of the fuel. 5-aminotetrazole nitrate has a less negative oxygen balance than typical nonazide fuels and is considered to be self-flagrating. This allows for compositions with significantly less PSAN (or other oxidizer) which will ignite more readily and combust at lower inflator operating pressures than previously known smokeless gas generators. Essentially, these compositions combine the benefits of the typical high-solids nonazide gas generators as exemplified by Poole (high burn rate, easily ignitable, low inflator operating pressures) with the benefits of PSAN-based smokeless nonazide gas generators (90–100% gas conversion, minimal solids). The result is an inflator that is smaller, lighter, cheaper and less complex in design. NQ indicates nitroguanidine. Other well known gas generator compositions may also be used in accordance with the present invention. See the Background of the Invention, for example.

In yet another aspect of the invention, a method of formulating gas generator compositions containing 5-ATN is described. The constituents of the gas generator compositions may all be obtained from suppliers well known in the art. In general, the base fuel (5AT) and any oxidizers are added to excess concentrated nitric acid and stirred until a damp paste forms. This paste is then formed into granules by either extrusion or forcing the material through a screen. The wet granules are then dried.

The nitric acid can be the standard reagent grade (1 5.9M, ~70 wt. % HNO<sub>3</sub>) or can be less concentrated as long as enough nitric acid is present to form the mononitrate salt of 5AT. The nitric acid should be chilled to 0–20° C. before adding the 5AT and oxidizers to ensure that the 5AT does not decompose in the concentrated slurry. When mixing the 5AT and oxidizers in the nitric acid medium, the precise mixing equipment used is not important—it is necessary however to thoroughly mix all the components and evaporate the excess nitric acid. As with any process using acids, the materials of construction must be properly selected to prevent corrosion. In addition to routine safety practices, sufficient ventilation and treatment of the acid vapor is important.

After forming a wet paste as described above, several methods can be used to form granules. The paste can be placed in a screw-feed extruder with holes of desired diameter and then chopped into desired lengths. An oscillating granulator may also be used to form granules of desired size. The material should be kept wet through all the processing steps to minimize safety problems. The final granules can be dried in ambient pressure or under vacuum. It is most preferred to dry the material at about 30° C. under a -1 2 psig vacuum. Example 15 illustrates the process.

## EXAMPLE 15

100 ml of concentrated nitric acid (15.9M, Reagent, Grade from Aldrich) was added to a glass-lined, stirred, and 15 jacketed vessel and cooled to 0° C. 100 g of dry SAT (Nippon Carbide), 58 g of dry AN (Aldrich ACS Grade), and 6.5 g of dry KN (Aldrich ACS Grade) were then added to form a slurry in nitric acid. As the mixture was stirred, the excess nitric acid evaporated, leaving a doughy paste consisting of a homogeneous mixture of 174 g 5AT nitrate, 64.5 g PSAN10, and a small amount of nitric acid. This material was then passed through a low-pressure extruder to form long “noodles” that were consequently chopped to from cylindrical granules. These granules were then placed in a 25 vacuum oven at 30° C. and -12 psig vacuum overnight. After drying, the granules were screened and those that passed through a No. 4 mesh screen and were retained on a No. 20 mesh screen and kept.

A preferred method of formulating gas generator compositions containing 5-aminotetrazole nitrate and phase stabilized ammonium nitrate is described in Example 16. One of ordinary skill will readily appreciate that the following description merely illustrates, but does not limit, mixing of the constituents in the exact amounts of ingredients 30 described. For example, other oxidizers may be used in lieu of PSAN.

## EXAMPLE 16

100 ml of 70 wt. % HNO<sub>3</sub> solution equals 99.4 g (1.58 40 mol) HNO<sub>3</sub> plus 42.69 (2.36 mol) H<sub>2</sub>O. The solution is mixed by stirring in 100 g dry 5-aminotetrazole (5-AT) which equals 1.18 mol 5-AT, 58 g dry ammonium nitrate (AN), and 6.5 g potassium nitrate (KN) (10% of total AN+KN). The sequence of addition is not critical. As mixing 45 occurs, 5-AT is converted into a nitric acid salt: 5-AT(1.18 mol=100 g)+HNO<sub>3</sub> (1.18 mol=74.4 g)=5-AT·HNO<sub>3</sub>. The AN and KN dissolve in the water present. Excess HNO<sub>3</sub> (99.4 g-74.4 g=25 g) and H<sub>2</sub>O (42.6 g) evaporate as the 50 mixture is stirred. As this occurs, AN (58 g) and KN(6.5 g) coprecipitate to form PSAN10 (64.5 g). Meanwhile, the 5-AT·HNO<sub>3</sub> formed while mixing is intimately mixed with the PSAN10. After mixing is complete, the end result is an intimate mixture of 174 g of 5-AT·HNO<sub>3</sub>+64.5 g PSAN10 with a small amount of HNO<sub>3</sub> and H<sub>2</sub>O to keep the mixture in a doughy or pasty form. Although potassium nitrate has been used to stabilize the ammonium nitrate, one of ordinary skill will readily appreciate that the ammonium nitrate may also be stabilized with other known stabilizers such as, but not limited to, potassium perchlorate and other potassium salts.

55 Granules or pellets are then formed from the paste by methods well known in the art. The granules or pellets are then dried to remove any residual HNO<sub>3</sub> and H<sub>2</sub>O. The end product consists of dry granules or pellets of a composition containing about 73 wt. % 5-AT·HNO<sub>3</sub>+27 wt. % PSAN10.

60 One of ordinary skill in the art will readily appreciate that the various amounts of the constituents described above can

## 11

be varied to alter the combustion and ballistic properties of the gas generant compositions.

Although the components of the present invention have been described in their anhydrous form, it will be understood that the teachings herein encompass the hydrated forms as well. While the foregoing examples illustrate and describe the use of the present invention, they are not intended to limit the invention as disclosed in certain preferred embodiments herein. Therefore, variations and modifications commensurate with the above teachings and the skill and/or knowledge of the relevant art, are within the scope of the present invention.

We claim:

1. A gas generant composition comprising a mixture of: a fuel consisting of 5-aminotetrazole nitrate; and

at least one oxidizer selected from the group consisting of phase stabilized ammonium nitrate; alkali metal and alkaline earth metal nitrates, nitrites, perchlorates, chlorates, and chlorites; and, alkali, alkaline earth, and transitional metal oxides,

wherein the 5-aminotetrazole nitrate is employed in a concentration of 55 to 85% by weight of the gas generant composition, and the oxidizer is employed in a concentration of 20 to 45% by weight of the gas generant.

2. The composition of claim 1 further comprising an inert combination slag former, binder, processing aid, and coolant selected from the group consisting of silicon, silicates, diatomaceous earth, clay, diatomaceous earth, and oxides such as alumina, silica, glass, and titania, wherein said inert slag former is employed in a concentration of 0.1 to 20% by weight of the gas generant composition.

3. The composition of claim 1 wherein the oxidizer is selected from the group consisting of phase stabilized ammonium nitrate, potassium nitrate, and strontium nitrate.

4. A gas generant composition comprising a mixture of a fuel consisting of 5-aminotetrazole nitrate; and

phase stabilized ammonium nitrate,

wherein 5-aminotetrazole nitrate is employed in a concentration of 30 to 95% by weight of the gas generant

## 12

composition, and phase stabilized ammonium nitrate is employed in a concentration of 5 to 70% by weight of the gas generant composition.

5. A gas generant composition wherein 5-aminotetrazole nitrate is employed in a concentration of about 73% by weight of the gas generant composition, and phase stabilized ammonium nitrate is employed in a concentration of about 27% by weight of the gas generant composition.

6. The composition of claim 5 wherein 5-aminotetrazole nitrate is employed in a concentration of about 73.12% by weight of the gas generant composition, and phase stabilized ammonium nitrate is employed in a concentration of about 26.88% by weight of the gas generant composition.

7. The composition of claim 4 further comprising an inert combination slag former, binder, processing aid, and coolant selected from the group consisting of silicon, silicates, diatomaceous earth, clay, and oxides such as alumina, silica, glass, and titania, wherein said inert slag former is employed in a concentration of 0.1 to 20% by weight of the gas generant composition.

8. A gas generant composition consisting essentially of a mixture of:

a fuel consisting of 5-aminotetrazole nitrate; and  
phase stabilized ammonium nitrate,

wherein 5-aminotetrazole nitrate is employed in a concentration of 30 to 95% by weight of the gas generant composition, and phase stabilized ammonium nitrate is employed in a concentration of 5 to 70% by weight of the gas generant composition.

9. A gas generant composition consisting of a mixture of:  
a fuel consisting of 5-aminotetrazole nitrate; and  
phase stabilized ammonium nitrate,

wherein 5-aminotetrazole nitrate is employed in a concentration of 30 to 95% by weight of the gas generant composition, and phase stabilized ammonium nitrate is employed in a concentration of 5 to 70% by weight of the gas generant composition.

\* \* \* \* \*